

# UNITED STATES PATENT OFFICE.

ERNST WOLFGANG KÜTTNER, OF BERLIN, GERMANY.

## PROCESS OF PRODUCING AND PROTECTING INSULATING-COVERINGS OF OXID ON WIRES, BANDS, &c.

1,137,986.

Specification of Letters Patent.

Patented May 4, 1915.

No Drawing.

Application filed September 2, 1910. Serial No. 580,198.

*To all whom it may concern:*

Be it known that I, DR. ERNST WOLFGANG KÜTTNER, engineer, citizen of Germany, subject of the King of Prussia and Emperor of 5 Germany, residing at Berlin, in the Kingdom of Prussia and Empire of Germany, have invented new and useful improvements in processes of producing and protecting insulating coverings of oxid on wires, bands, 10 bundles, or coils, particularly of aluminium and its alloys, of which the following is a specification.

It is known that on naked metallic wires and bands a covering of oxid can be produced, which serves in many instances as a 15 sufficient electric insulation. On aluminium wires a well insulating covering of oxid will form by itself. But the insulation obtained by such means is not uniform and durable, 20 particularly if the oxidized wires are subsequently to be wound into coils. For the purpose of producing coverings of oxid on naked metallic wires or bands, particularly such of greater section, which are intended 25 to be wound in coils or solenoids, an oxidizing medium is made to act in such a manner that a close contact is obtained between the said oxidizing medium and all parts of the metallic surface. This process is to be particularly employed for aluminium and its 30 alloys. The completed coil wound of naked wire may also be exposed to the action of the oxidizing medium. Instead of oxid the insulating layers may consist of other chemical 35 compounds (as for instance salts) of the metal.

The coverings of oxid, hydroxid or salt produced by one of the hereinbefore described methods are still very easily affected 40 by friction or pressure or the like.

With the object of protecting them against the effects of pressure during their finishing process, transport and installation and use the present invention provides that a suitable protective coating is brought upon such 45 treated metallic surface. With coils such protective coating or filling is introduced into the interior of the coils and between the individual turns. This covering may 50 according to circumstances be arranged only after the coils have been completed and even after they have been bound (bandaged). In doing so it will be preferable to employ a vacuum or a pressure, so as to allow of the 55 filling material penetrating more deeply

through the bandages into the interior of the coil. In most instances it will, however, be advisable, to introduce the filling into the coil before the latter is bound, as the filling will then also help to compensate or render 60 harmless the frictional pressure produced in binding. If a suitable protecting medium is employed, the coils may be also treated with it already during the oxidizing process. Preferably the filling may consist of a liquid, 65 which will, after cooling or by evaporation, become sufficiently solid and dry. So a material which will melt under the influence of heat, as wax, resin, pitch, india-rubber or the like may be introduced into a coil 70 heated to a sufficiently high temperature. For the purpose of obtaining a thorough penetration a vacuum or an overpressure may be employed. In many instances it will suffice to simply dip the coil into the molten 75 medium. On the other hand a solution in alcohol or benzine or the like may be employed, such as varnish, rubber-solution or the like. Also these may be introduced into the coils by a dipping process, either in a 80 cold or hot state or by impregnation either in a vacuum or under pressure. In the last mentioned instance the drying and evaporation of the solvent may be accelerated by heating. On the coils being heated, a better 85 distribution or penetration of many mediums will be obtained, and for the purpose of improving this effect the finished or half finished coils may be heated either once or several times. Such protective mediums 90 may, provided they are pliable or soft, also be applied to the oxidized wires before the same are wound into coils; in such instance the wires will be oxidized in their raw state say in bundles or rings and are wound into 95 coils while being simultaneously provided with the soft protective covering. It is obvious, that the filling medium should then be tough and adhesive, so that it is not squeezed out by the winding operation and 100 will not flake off.

If a substance is employed as protective medium, which will have an oxidizing effect on the metal, the covering of oxid may be further increased by the action of the 105 protective medium. As such protective medium may be employed oxidizing varnishes, which are varnishes having an acid or alkalic reaction. For instance, such often occurs in the trade oil varnishes containing 110

free oleic acid or prepared with rancid oils. These varnishes are ordinarily avoided in the treatment of metals, as they attack them, but here, this effect is useful. Further, varnishes are well-known which are prepared with tar or phenols having an acid reaction or acid fats and oils and all kinds of paints which contain free acids or alkalis, as for instance, oil colors prepared with rancid 10 oils. Also varnishes or paints of an otherwise neutral character may be converted into an oxidizing medium, by adding to them an oxidizing substance or applying such oxidizing substance to the surface of the wires 15 besides the paint. The coils or wires may be treated with an oxidizing liquid or an oxidizing vapor and, be covered while still moist with the protective covering, so that the oxidizing medium will for some time 20 still continue its oxidizing effect under the protective covering. The oxidizing medium may thereby mix with the protective medium. If an aluminium wire or coil is moistened with water and then saturated with 25 any varnish, preferably at a raised temperature, a covering of oxid will be gradually produced and will increase in thickness until the water will have disappeared beneath the 30 coat of varnish, which may be preferably obtained by artificial drying.

The protective covering need not entirely fill out the coils; it will, in many instances be quite sufficient if the outer turns are penetrated by the subsequently hardening 35 protective medium, so that a sort of crust is formed, which will receive the outside pressure and distribute it over larger surfaces of the coil. It is not absolutely necessary, for the protective covering to consist 40 of an insulating material, as the insulation proper of the wires is produced by the covering of oxid and the filling medium has the object only to afford a mechanical protection for the covering of oxid.

45 Having now particularly described and ascertained the nature of my said invention, and in what manner the same is to be performed, I declare that what I claim is:

50 1. A process for producing electric coils comprising the steps of winding a wire containing aluminum and of any shape into coils, oxidizing the entire surface of said wire after it is coiled, and covering the oxidized surface with a mechanically resistant 55 coating adapted to protect said oxidized surface against the damages of pressure.

2. A process for producing electric coils comprising the steps of winding into coils a wire containing aluminum and of any shape, 60 oxidizing the entire surface of said wire after it is coiled and covering the oxidized surface with a mechanically resistant coating adapted to protect said oxidized surface 65 against the damages of pressure, said coating being introduced in a liquid state into

the interior of the coil and between the individual turns.

3. A process for producing electric coils comprising the steps of winding into coils a wire containing aluminum and of any shape, 70 oxidizing the entire surface of said wire, and covering the oxidized surface with a mechanically resistant coating adapted to protect said oxidized surface against the damages of pressure, said coating being introduced in a liquid state into the interior of 75 the coil and between the individual turns during the oxidizing process.

4. A process for producing electric coils comprising the steps of winding a wire containing aluminum and of any shape into coils, oxidizing the entire surface of said wire after it is coiled, and covering the oxidized surface with a mechanically resistant coating adapted to protect said oxidized 80 surface against the damages of pressure, 85 said coating consisting of a solution with an evaporable solvent, said coating being introduced in a liquid state into the interior of the coil and between the individual turns.

5. A process for producing and protecting insulating coverings of oxid on metallic wires of any shape containing aluminum and in the form of bundles or coils, which consists in oxidizing the entire surface and 90 covering it with a solidifying and drying protective liquid, said liquid being introduced into the interior of the coil and between the individual turns, said coil being subsequently heated an optional number of 95 times.

6. A process for producing and protecting insulating coverings of oxid on wires, or bands, particularly of aluminum and its alloys, which consists in treating the surface of the metal in all parts with an oxidizing medium, the oxid produced being protected by a coating consisting of a liquid which will become sufficiently solid and dry 105 before the insulating wires are exposed to friction or pressure, said coating having oxidizing properties, while it still remains liquid.

7. A process for producing and protecting insulating coverings of oxid on wires or bands particularly of aluminum and its alloys, which consists in treating the surface of the metal in all parts with a solidifying and drying liquid having oxidizing properties and which on becoming sufficiently solid and dry forms a protective coating on the oxidized metallic surface before the wires are exposed to friction or pressure.

8. A process for producing and protecting insulating coverings of oxid on wires, bands, bundles or coils, particularly of aluminum and its alloys consisting in treating the surface of the metal in all parts with an oxidizing medium, a protective coating 125 being applied to said metallic surfaces while 130

the oxidizing medium on said metallic surfaces is yet active, the said protective coating and the oxidizing medium being both applied in a moist state.

- 5 9. A process for producing and protecting insulating coverings of oxid on wires, bands, bundles or coils, particularly of aluminum and its alloys, consisting in treating the surface of the metal in all parts with an oxidizing medium, a protective coating being applied to said metallic surface while the oxidizing medium on said metallic surface is yet active, the said protective coating and the oxidizing medium being both applied in
- 10 a moist state and accelerating the drying process by heating.
- 15 10. A process for producing and protect-

ing insulating coverings of oxid on bundles or coils of metallic wire, particularly of aluminum and its alloys, consisting in treating the surface of the metal in all parts with an oxidizing medium, a protective coating being introduced into the interior of the bundles and coils and between the individual turns, said protective coating penetrating only the outer turns of said bundles or coils.

In testimony whereof I have hereunto set my hand in presence of two subscribing witnesses.

DR. ERNST WOLFGANG KÜTTNER.

Witnesses:

WOLDEMAR HAUPT,  
BRUNO BRUER.